



US010543536B2

(12) **United States Patent**  
**Kim et al.**

(10) **Patent No.:** **US 10,543,536 B2**  
(45) **Date of Patent:** **Jan. 28, 2020**

(54) **METHOD FOR FABRICATING METAL NANOPARTICLES**

(71) Applicant: **LG CHEM, LTD.**, Seoul (KR)

(72) Inventors: **Kwanghyun Kim**, Daejeon (KR); **Gyo Hyun Hwang**, Daejeon (KR); **Sang Hoon Kim**, Daejeon (KR); **Jun Yeon Cho**, Daejeon (KR)

(73) Assignee: **LG CHEM, LTD.**, Seoul (KR)

(\*) Notice: Subject to any disclaimer, the term of this patent is extended or adjusted under 35 U.S.C. 154(b) by 1104 days.

(21) Appl. No.: **14/892,920**

(22) PCT Filed: **Jun. 3, 2014**

(86) PCT No.: **PCT/KR2014/004935**

§ 371 (c)(1),

(2) Date: **Nov. 20, 2015**

(87) PCT Pub. No.: **WO2014/196786**

PCT Pub. Date: **Dec. 11, 2014**

(65) **Prior Publication Data**

US 2016/0114398 A1 Apr. 28, 2016

(30) **Foreign Application Priority Data**

Jun. 7, 2013 (KR) ..... 10-2013-0065441

(51) **Int. Cl.**

**B22F 1/00** (2006.01)  
**B22F 9/00** (2006.01)

(Continued)

(52) **U.S. Cl.**  
CPC ..... **B22F 9/24** (2013.01); **B22F 1/0003** (2013.01); **B22F 1/0007** (2013.01); **B22F 1/007** (2013.01);

(Continued)

(58) **Field of Classification Search**  
CPC .... B22F 1/0007; B22F 1/0011; B22F 1/0014; B22F 1/0018; B22F 1/0048; B22F 1/0051;

(Continued)

(56) **References Cited**

**U.S. PATENT DOCUMENTS**

6,660,058 B1 \* 12/2003 Oh ..... B22F 1/0018 75/351  
2008/0096986 A1 \* 4/2008 Thomazeau ..... B01J 23/42 518/716

(Continued)

**FOREIGN PATENT DOCUMENTS**

CN 1476413 A 2/2004  
CN 102245333 A 11/2011

(Continued)

**OTHER PUBLICATIONS**

Sun. Platinum catalyzed growth of NiPt hollow spheres with an ultrathin shell. J. Mater. Chem., 2011, 21, 1925-1930 (Year: 2011).\*

(Continued)

*Primary Examiner* — Matthew E. Hoban

(74) *Attorney, Agent, or Firm* — Dentons US LLP

(57) **ABSTRACT**

The present specification relates to a method for fabricating metal nanoparticles.

**23 Claims, 17 Drawing Sheets**



(51) **Int. Cl.**  
**B22F 9/06** (2006.01)  
**B22F 9/16** (2006.01)  
**B22F 9/24** (2006.01)

(52) **U.S. Cl.**  
CPC ..... **B22F 1/0018** (2013.01); **B22F 1/0044** (2013.01); **B22F 1/0048** (2013.01); **B22F 2009/245** (2013.01); **B22F 2304/054** (2013.01)

(58) **Field of Classification Search**

CPC ..... B22F 2001/0033; B22F 2001/0037; B22F 9/00; B22F 9/06; B22F 9/16; B22F 9/18; B22F 9/20; B22F 9/24; B22F 9/26; B22F 2009/165; B22F 2009/245

See application file for complete search history.

(56) **References Cited**

U.S. PATENT DOCUMENTS

|                 |         |                     |
|-----------------|---------|---------------------|
| 2008/0166259 A1 | 7/2008  | Kijima et al.       |
| 2009/0283726 A1 | 11/2009 | Mizoguchi et al.    |
| 2010/0143184 A1 | 6/2010  | Niidome et al.      |
| 2011/0283834 A1 | 11/2011 | Hight-Walker et al. |
| 2011/0311635 A1 | 12/2011 | Stucky et al.       |
| 2012/0015211 A1 | 1/2012  | Gu et al.           |
| 2012/0037041 A1 | 2/2012  | Nolte et al.        |
| 2012/0321897 A1 | 12/2012 | Yang et al.         |

FOREIGN PATENT DOCUMENTS

|    |                   |         |
|----|-------------------|---------|
| JP | 2006-45582 A      | 2/2006  |
| JP | 2006278312 A      | 10/2006 |
| JP | 2009057311 A      | 3/2009  |
| KR | 10-2003-0008763 A | 1/2003  |
| KR | 10-2003-0072549 A | 9/2003  |
| KR | 10-2010-0026115 A | 3/2010  |
| WO | 0242201 A1        | 5/2002  |

OTHER PUBLICATIONS

Zhao, Y., et al., "Methanol electro-oxidation on Ni@Pd core-shell nanoparticles supported on multi-walled carbon nanotubes in alkaline media," International Journal of Hydrogen Energy, vol. 35,2010, pp. 3249-3257.

Ahmed et al., "Bimetallic Cu—Ni nanoparticles of varying composition (CuNi<sub>3</sub>, CuNi, Cu<sub>3</sub>Ni)," Colloids and Surfaces A: Physicochem. Eng. Aspects 331(3): 206-212 (2008).

Weihua et al., "Synthesis and characterization of Pt—Cu bimetallic alloy nanoparticles by reverse micelles method," Colloids and Surfaces A: Physicochem. Eng. Aspects 273(1-3): 35-42 (2006).

Pal et al., "Shape controlled synthesis of iron-cobalt alloy magnetic nanoparticles using soft template method," Materials Letters 64(10): 1127-1129 (2010).

\* cited by examiner

[Figure 1]



[Figure 2]



[Figure 3]



[Figure 4]



[Figure 5]



[Figure 6]



[Figure 7]



[Figure 8]



[Figure 9]



[Figure 10]



[Figure 11]



[Figure 12]



[Figure 13]



[Figure 14]



[Figure 15]



[Figure 16]



[Figure 17]



[Figure 18]



[Figure 19]



[Figure 20]



[Figure 21]



[Figure 22]



## 1

## METHOD FOR FABRICATING METAL NANOPARTICLES

## TECHNICAL FIELD

This application is a National Stage Application of International Application No. PCT/KR2014/004935, filed on Jun. 3, 2014, which claims the benefit of Korean Patent Application No. 10-2013-0065441, filed on Jun. 7, 2013, all of which are hereby incorporated by reference in their entirety for all purposes as if fully set forth herein.

The present specification relates to a method for fabricating metal nanoparticles.

## BACKGROUND ART

Nanoparticles are particles having nanoscale particle sizes, and show optical, electrical and magnetic properties completely different from those of bulk materials due to a large specific surface area and the quantum confinement effect, in which energy required for electron transfer changes depending on the size of material. Accordingly, due to such properties, much interest has been concentrated on their applicability in the catalytic, electromagnetic, optical, medical fields, and the like. Nanoparticles may be considered as intermediates between bulks and molecules, and may be synthesized in terms of two approaches, that is, the “top-down” approach and the “bottom-up” approach.

Examples of a method for synthesizing a metal nanoparticle include a method for reducing metal ions in a solution by using a reducing agent, a method for synthesizing a metal nanoparticle using gamma-rays, an electrochemical method, and the like, but in the existing methods, it is difficult to synthesize nanoparticles having a uniform size and shape, or it is difficult to economically mass-produce high-quality nanoparticles for various reasons such as problems of environmental contamination, high costs, and the like by using organic solvents.

Meanwhile, in order to prepare metal nanoparticles in the related art, metal nanoparticles have been prepared by synthesizing particles with a low reduction potential, such as Ag, Cu, Co, and Ni, substituting the surface of particles, such as Ag, Cu, Co, and Ni with a metal having a higher reduction potential than the particles, for example, Pt, Pd, or Au by a potential difference substitution method, and after the surface substitution, melting Ag, Cu, Co, Ni, and the like remaining inside the particles through an acid treatment. In this case, there is a problem in the process in that a post-treatment needs to be performed with an acid, and since the potential difference substitution method is a natural reaction, there are few factors that may control the post-treatment, and thus it is difficult to prepare uniform particles. Therefore, there is a need for a method for easily preparing uniform metal nanoparticles.

## DETAILED DESCRIPTION OF THE INVENTION

## Technical Problem

The present specification has been made in an effort to provide a method for fabricating metal nanoparticles, which generates no environmental pollution and is capable of easily implementing mass production with low costs.

Further, the present specification has been made in an effort to provide a method for fabricating metal nanoparticles, which has enhanced activity due to a large specific surface area.

## 2

The problems of the present specification to be solved by the present specification are not limited to the aforementioned technical problems, and other technical problems, which have not been mentioned, may be obviously understood by a person with ordinary skill in the art from the following description.

## Technical Solution

10 An exemplary embodiment of the present specification provides a method for fabricating metal nanoparticles, the method including: forming a solution including: a solvent; a first metal salt which provides a first metal ion or an atomic group ion including the first metal ion in the solvent; a second metal salt which provides a second metal ion or an atomic group ion including the second metal ion in the solvent; a first surfactant which forms micelles in the solvent; and a second surfactant which forms micelles together with the first surfactant in the solvent; and forming the metal nanoparticle by adding a reducing agent to the solution.

15 20 25 An exemplary embodiment of the present specification provides a metal nanoparticle prepared by the preparation method.

## Advantageous Effects

30 35 The method for fabricating metal nanoparticles according to the present specification is advantageous in that it is possible to mass-produce metal nanoparticles having a uniform size of several nanometers, there is a cost reduction effect, and no environmental pollution is generated in the preparation process. Furthermore, according to the method for fabricating metal nanoparticles according to the present specification, it is possible to prepare a metal nanoparticle which has enhanced activity due to a large specific surface area enhanced activity.

40 45 Further, according to a metal nanoparticle prepared by the preparation method of the present specification, the inner surface area of a shell may be utilized as a contact area, and thus, there is an advantage in that when the metal nanoparticle is included in a catalyst, the catalyst efficiency is enhanced.

## BRIEF DESCRIPTION OF DRAWINGS

50 FIGS. 1 to 5 illustrate an example of micelles according to an exemplary embodiment of the present specification.

55 FIGS. 6 and 7 illustrate an example, in which a metal ion forming a shell portion of metal nanoparticle or an atomic group ion including the metal ion is positioned in a micelle, according to an exemplary embodiment of the present specification.

60 FIG. 8 illustrates an electron transmission microscope (TEM) image of the metal nanoparticles prepared according to Example 1.

65 FIG. 9 illustrates an electron transmission microscope (TEM) image of the metal nanoparticles prepared according to Example 2.

FIG. 10 illustrates an electron transmission microscope (TEM) image of the metal nanoparticles prepared according to Example 3.

65 FIG. 11 illustrates an electron transmission microscope (TEM) image of the metal nanoparticles prepared according to Example 4.

FIG. 12 illustrates an electron transmission microscope (TEM) image of the metal nanoparticles prepared according to Example 5.

FIG. 13 illustrates an electron transmission microscope (TEM) image of the metal nanoparticles prepared according to Example 6.

FIGS. 14 and 15 illustrate an electron transmission microscope (TEM) image of the metal nanoparticles prepared according to Example 7.

FIG. 16 illustrates an electron transmission microscope (TEM) image of the metal nanoparticles prepared according to Example 8.

FIG. 17 illustrates an electron transmission microscope (TEM) image of the metal nanoparticles prepared according to Example 9.

FIG. 18 illustrates an electron transmission microscope (TEM) image of the metal nanoparticles prepared according to Example 10.

FIGS. 19 and 20 illustrate an electron transmission microscope (TEM) image of the metal nanoparticles prepared according to Example 11.

FIGS. 21 and 22 illustrate an electron transmission microscope (TEM) image of the metal nanoparticles prepared according to Example 12.

#### BEST MODE

The benefits and features of the present application, and the methods of achieving the benefits and features will become apparent with reference to exemplary embodiments to be described below in detail along with the accompanying drawings. However, the present application is not limited to the exemplary embodiments to be disclosed below, but may be implemented in various other forms, and the present exemplary embodiments are provided for rendering the disclosure of the present application complete and for fully representing the scope of the invention to a person with ordinary skill in the technical field to which the present application pertains, and the present application will be defined only by the scope of the claims. The size and relative size of the constituent element illustrated in the drawing may be exaggerated for the clarity of description.

Unless otherwise defined in the present specification, all the terms (including technical and scientific terms) used in the present specification will be able to be used as a meaning which may be commonly understood to a person with ordinary skill in the technical field to which the present specification pertains. Further, the terms defined in a dictionary generally used are not interpreted ideally or excessively unless the terms have been clearly and specially defined.

Hereinafter, the present specification will be described in more detail.

An exemplary embodiment of the present specification provides a method for fabricating metal nanoparticles, the method including: forming a solution including: a solvent; a first metal salt which provides a first metal ion or an atomic group ion including the first metal ion in the solvent; a second metal salt which provides a second metal ion or an atomic group ion including the second metal ion in the solvent; a first surfactant which forms micelles in the solvent; and a second surfactant which forms micelles together with the first surfactant in the solvent; and forming the metal nanoparticle by adding a reducing agent to the solution.

According to an exemplary embodiment of the present specification, a hollow core may be formed inside of the metal nanoparticle by the preparation method.

In the present specification, the term "hollow" means that the core portion of the metal nanoparticle is empty. Further, the term "hollow" may be used as the same meaning as a hollow core. The term "hollow" may include a term such as a hollow, a hole, and a void.

According to an exemplary embodiment of the present specification, the hollow may include a space in which the internal material is not present by 50% by volume or more, specifically 70% by volume or more, and more specifically 80% by volume or more. Alternatively, the hollow may also include a space of which the inside is empty by 50% by volume or more, specifically 70% by volume or more, and more specifically 80% by volume or more. Alternatively, the hollow may include a space having an internal porosity of 50% by volume or more, specifically 70% by volume or more, and more specifically 80% by volume or more.

According to an exemplary embodiment of the present specification, the preparation method may include that the inner region of the micelle formed by the first surfactant is formed of a hollow.

The method for fabricating metal nanoparticles according to an exemplary embodiment of the present specification does not use the reduction potential difference and thus has an advantage in that the reduction potential between the first metal ion and the second metal ion, which form shells, is not considered. The preparation method of the present specification uses charges among metal ions and thus is simpler than the methods for preparing a metal nanoparticle, which uses the reduction potential difference in the related art. Therefore, the method for fabricating metal nanoparticles according to the present specification facilitates the mass production, and may prepare the metal nanoparticle at low costs. Furthermore, the method does not use the reduction potential difference and thus has an advantage in that various metal salts may be used because the limitation of the metal salt to be used is reduced as compared to the methods for preparing a metal nanoparticle in the related art.

According to an exemplary embodiment of the present specification, the forming of the solution may include forming, by the first and second surfactants, micelles in a solution.

According to an exemplary embodiment of the present specification, in the preparation method, the first metal ion or the atomic group ion including the first metal ion; and the second metal ion or the atomic group ion including the second metal ion may form a shell portion of the metal nanoparticle.

According to an exemplary embodiment of the present specification, the first metal ion or the atomic group ion including the first metal ion has a charge which is opposite to a charge at the outer end portion of the first surfactant, and the second metal ion or the atomic group ion including the second metal ion may have a charge which is the same as the charge at the outer end portion of the first surfactant.

Therefore, the first metal ion or the atomic group ion including the first metal ion is positioned at the outer end portion of the first surfactant which forms micelles in the solution, thereby producing a form which surrounds the outer surface of the micelle. Furthermore, the second metal ion or the atomic group ion including the second metal ion surrounds the outer surface of the first metal ion or the atomic group ion including the first metal ion. The first metal

salt and the second metal salt may form a shell portion including the first metal and the second metal, respectively, by a reducing agent.

The outer end portion of the surfactant in the present specification may mean the outer side portion of the micelle of the first or second surfactant which forms the micelle. The outer end portion of the surfactant of the present specification may mean the head of the surfactant. Further, the outer end portion of the present specification may determine the charge of the surfactant.

In addition, the surfactant of the present specification may be classified into an ionic surfactant or a non-ionic surfactant depending on the type of the outer end portion, and the ionic surfactant may be a cationic surfactant, an anionic surfactant, a zwitterionic surfactant or an amphoteric surfactant. The zwitterionic surfactant contains both positive and negative charges. If the positive and negative charges in the surfactant of the present specification are dependent on the pH, the surfactant may be an amphoteric surfactant, which may be zwitterionic in a certain pH range. Specifically, the anionic surfactant in the present specification may mean that the outer end portion of the surfactant is negatively charged, and the cationic surfactant may mean that the outer end portion of the surfactant is positively charged.

According to an exemplary embodiment of the present specification, in the metal nanoparticle prepared by the preparation method, a cavity may be formed in one or more regions of the shell portion.

The cavity of the present specification may mean an empty space which is continuous from one region of the outer surface of the metal nanoparticle. The cavity of the present specification may be formed in the form of one tunnel from one region of the outer surface of the shell portion. The tunnel form may be a straight line, a continuous form of a curve or a straight line, and a continuous form in which a curve and a straight line are mixed.

According to an exemplary embodiment of the present specification, when the metal nanoparticle includes a hollow, the cavity may be an empty space extending from the outer surface of the shell portion to the hollow.

Further, according to an exemplary embodiment of the present specification, when the metal nanoparticle does not include a hollow, the cavity may be any empty space which is continuous from the outer surface of the shell portion to an inner or outer region of the metal nanoparticle. Specifically, when the metal nanoparticle does not include a hollow, the cavity may be an empty space extending from one region of the shell portion to one inner region of the metal nanoparticle, and may also be an empty space extending from one region of the shell portion to another region of the shell portion.

Further, according to an exemplary embodiment of the present specification, when the metal nanoparticle includes one or more bowl-type particles, the cavity may also mean an empty space which does not form a shell portion.

The cavity of the present specification may serve to utilize the inner surface area of the metal nanoparticle. Specifically, when the metal nanoparticle is used for a use such as a catalyst, the cavity may serve to increase a surface area which may be brought into contact with the reactant. Therefore, the cavity may serve to exhibit high activity of the metal nanoparticle.

According to an exemplary embodiment of the present specification, the shell portion may mean a region of the nanoparticle including the metal. Specifically, the shell portion may mean a region of the metal particle except for the hollow and the cavity.

According to an exemplary embodiment of the present specification, the metal nanoparticle prepared by the preparation method may be a nanoparticle having a spherical shape.

5 The spherical shape in the present specification does not mean only a perfect spherical shape, and may include a roughly spherical shape. For example, in the hollow metal nanoparticle, the outer surface having a spherical shape may not be smooth, and the radius of curvature in one hollow metal nanoparticle may not be constant.

According to an exemplary embodiment of the present specification, the metal nanoparticle prepared by the preparation method may be a metal nanoparticle including an inner hollow and one or two or more cavities.

15 Further, according to an exemplary embodiment of the present specification, the metal nanoparticle prepared by the preparation method may be a metal nanoparticle including one or two or more cavities without an inner hollow.

According to an exemplary embodiment of the present specification, 20 the metal nanoparticle prepared by the preparation method may be in the form of one bowl-type particle or in the form in which two or more bowl-type particles are partially brought into contact with each other.

The metal nanoparticle of the present specification in the form of the bowl-type particle or in the form in which two or more bowl-type particles are partially brought into contact with each other may mean that the size of the cavities occupies 30% or more of the entire shell portion.

Further, the metal nanoparticle in the form in which the 30 two or more bowl-type particles are partially brought into contact with each other may mean a form in which the cavities are continuously formed, and thus the metal nanoparticles are partially split.

In addition, the bowl-type particle may mean that the 35 cavities are continuously formed, and thus 30% or more of the surface of the nanoparticle does not form a shell portion.

The bowl type in the present specification may mean that 40 at least one curved line region is included on the cross section. Alternatively, the bowl type may mean that a curved line region and a straight line region are mixed on the cross section. Alternatively, the bowl type may be a semispherical shape, and the semispherical shape may not be necessarily a form in which the particle is divided such that the division line passes through the center of the sphere, but may be a 45 form in which one region of the sphere is removed. Furthermore, the spherical shape does not mean only a perfect spherical shape, and may include a roughly spherical shape. For example, the outer surface of the sphere may not be smooth, and the radius of curvature of the sphere may not be constant. Alternatively, the bowl-type particle of the present specification may mean that a region corresponding to a 30% to 80% of the entire shell portion of the hollow nanoparticle is not continuously formed.

According to an exemplary embodiment of the present 50 specification, in the preparation method, a cavity may be formed in one or two or more regions of the shell portion by adjusting the concentration; the chain length; the size of the outer end portion; or the type of charge, of the second surfactant.

60 According to an exemplary embodiment of the present specification, the first surfactant may serve to form micelles in a solution to allow the metal ion or the atomic group ion including the metal ion to form a shell portion, and the second surfactant may serve to form the cavity of the metal nanoparticle.

According to an exemplary embodiment of the present specification, the preparation method may include forming

the shell portion of the metal nanoparticle in a micelle region which the first surfactant forms, and forming the cavity of the metal nanoparticle in a micelle region which the second surfactant forms.

According to an exemplary embodiment of the present specification, the forming of the solution may include adjusting the size or number of the cavities by varying the concentrations of the first and second surfactants. Specifically, according to an exemplary embodiment of the present specification, the molar concentration of the second surfactant may be 0.01 to 1 time the molar concentration of the first surfactant. Specifically, the molar concentration of the second surfactant may be 1/30 to 1 time the molar concentration of the first surfactant.

According to an exemplary embodiment of the present specification, the first surfactant and the second surfactant in the forming of the solution may form micelles depending on the concentration ratio. The size of the cavities or the number of the cavities in the metal nanoparticle may be adjusted by adjusting the molar concentration ratio of the first surfactant to the second surfactant. Furthermore, a metal nanoparticle including one or more bowl type particles may also be prepared by allowing the cavity to be continuously formed.

Further, according to an exemplary embodiment of the present specification, the forming of the solution may include adjusting the size of the cavity by adjusting the size of the outer end portion of the second surfactant.

In addition, according to an exemplary embodiment of the present specification, the forming of the solution may include forming a cavity in the second surfactant region by adjusting the chain length of the second surfactant to be different from the chain length of the first surfactant.

According to an exemplary embodiment of the present specification, the chain length of the second surfactant may be 0.5 to 2 times the chain length of the first surfactant. Specifically, the chain length may be determined by the number of carbon atoms.

According to an exemplary embodiment of the present specification, it is possible to allow a metal salt bonded to the outer end portion of the second surfactant not to form the shell portion of the metal nanoparticle by making the chain length of the second surfactant different from the chain length of the first surfactant.

Furthermore, according to an exemplary embodiment of the present specification, the forming of the solution may include forming a cavity by adjusting the charge of the second surfactant to be different from the charge of the first surfactant.

According to an exemplary embodiment of the present specification, a first metal ion or an atomic group ion including the first metal ion, which has a charge opposite to the first and second surfactants, may be positioned at the outer end portions of the first and second surfactants, which form micelles in the solvent. Further, the second metal ion opposite to the charge of the first metal ion may be positioned on the outer surface of the first metal ion.

FIGS. 6 and 7 illustrate an example, in which a metal ion and an atomic group ion including the metal ion are positioned at an outer end portion of the first surfactant, which forms micelles, according to an exemplary embodiment of the present specification.

According to an exemplary embodiment of the present specification, the first metal ion and the second metal ion, which are formed at the outer end portion of the first surfactant, may form the shell portion of the metal nanoparticle, and the first metal ion and the second metal ion,

which are positioned at the outer end portion of the second surfactant, do not form the shell and may form a cavity.

According to an exemplary embodiment of the present specification, when the first surfactant is an anionic surfactant, the first surfactant forms micelles in the forming of the solution, and the micelle may be surrounded by cations of the first metal ion or the atomic group ion including the first metal ion. Furthermore, the atomic group ion including the second metal ion of the anion may surround the cations.

10 Furthermore, in the forming of the metal nanoparticle by adding a reducing agent, the cations surrounding the micelle forms a first shell, and the anions surrounding the cations may form a second shell.

In addition, according to an exemplary embodiment of the present specification, when the first surfactant is a cationic surfactant, the first surfactant forms micelles in the forming of the solution, and the micelle may be surrounded by anions of the atomic group ion including the first metal ion. Furthermore, the second metal ion of the cation or the atomic group ion including the second metal ion on may surround the anions. Furthermore, in the forming of the metal nanoparticle by adding a reducing agent, the anions surrounding the micelle form a first shell, and the cations surrounding the anions may form a second shell.

15 According to an exemplary embodiment of the present specification, the forming of the metal nanoparticle may include forming the first and second surfactant regions, which form the micelles, with a hollow.

20 Further, according to an exemplary embodiment of the present specification, the forming of the metal nanoparticle may include filling the first and second surfactant regions, which form the micelles, with a metal. Specifically, when the chain length of the second surfactant is longer or shorter than the length of the first surfactant forming the micelle, the inside of the micelle may be filled with the first metal salt and the second metal salt.

25 According to an exemplary embodiment of the present specification, when the inside of the first and second surfactants is filled with a metal, it is possible to prepare a metal nanoparticle including one or two or more cavities without a hollow.

30 According to an exemplary embodiment of the present specification, both the first surfactant and the second surfactant may be a cationic surfactant.

35 Alternatively, according to an exemplary embodiment of the present specification, both the first surfactant and the second surfactant may be an anionic surfactant.

40 According to an exemplary embodiment of the present specification, when both the first surfactant and the second surfactant have the same charge, a micelle may be formed by making the chain length of the second surfactant different from the chain length of the first surfactant. FIG. 1 illustrates an example thereof.

45 Specifically, by a difference in chain lengths of the second surfactant, the first and second metal ions positioned at the outer end portion of the second surfactant are not adjacent to the first and second metal ions positioned at the outer end portion of the first surfactant, and thus, do not form the shell portion.

50 FIG. 1 illustrates an example of the cases where the first surfactant and the second surfactant have the same charge, according to an exemplary embodiment of the present specification.

55 According to an exemplary embodiment of the present specification, one of the first surfactant and the second surfactant may be an anionic surfactant, and the other may be a cationic surfactant. That is, in an exemplary embodiment,

ment of the present specification, the first and second surfactants may have charges different from each other.

According to an exemplary embodiment of the present specification, when the first and second surfactants have charges different from each other, the cavity of the metal nanoparticle may be formed by making the lengths of the chains different. In this case, the principle in which the cavity is formed is the same as the case where the above-described first and second surfactants have the same charge.

According to an exemplary embodiment of the present specification, when the first and second surfactants have charges different from each other, the cavity of the metal nanoparticle may be formed even though the lengths of the chains of the first and second surfactants are the same as each other. In this case, the outer end portion of the first surfactant, which is adjacent to the outer end portion of the second surfactant in the micelle, donates and accepts charges, and thus, is neutralized, so that the metal ion is not positioned. Therefore, the portion in which the metal ion is not positioned does not form a shell portion, thereby forming the cavity of the metal nanoparticle.

FIG. 4 illustrates an example, in which the first and second surfactants, which are differently charged, form micelles, according to an exemplary embodiment of the present specification.

According to an exemplary embodiment of the present specification, the first surfactant may be an anionic surfactant or a cationic surfactant, and the second surfactant may be a non-ionic surfactant.

According to an exemplary embodiment of the present specification, when the second surfactant is a non-ionic surfactant, the cavity of the metal nanoparticle may be formed because the metal ion is not positioned at the outer end portion of the second surfactant. Therefore, when the second surfactant is non-ionic, the cavity of the metal nanoparticle may be formed even when the length of the chain of the second surfactant is the same as or different from that of the first surfactant.

FIG. 2 illustrates an example of the cases where the second surfactant is a non-ionic surfactant, according to an exemplary embodiment of the present specification.

According to an exemplary embodiment of the present specification, the first surfactant may be an anionic surfactant or a cationic surfactant, and the second surfactant may be a zwitterionic surfactant.

According to an exemplary embodiment of the present specification, when the second surfactant is a zwitterionic surfactant, the cavity of the metal nanoparticle may be formed because the metal ion is not positioned at the outer end portion of the second surfactant. Therefore, when the second surfactant is zwitterionic, the cavity of the metal nanoparticle may be formed even when the length of the chain of the second surfactant is the same as or different from that of the first surfactant.

FIG. 3 illustrates an example of the cases where the second surfactant is a zwitterionic surfactant, according to an exemplary embodiment of the present specification.

The anionic surfactant of the present specification may be selected from the group consisting of ammonium lauryl sulfate, sodium 1-heptanesulfonate, sodium hexanesulfonate, sodium dodecyl sulfate, triethanol ammonium dodecylbenzenesulfate, potassium laurate, triethanolamine stearate, lithium dodecyl sulfate, sodium lauryl sulfate, alkyl polyoxyethylene sulfate, sodium alginate, dioctyl sodium sulfosuccinate, phosphatidylglycerol, phosphatidylinositol, phosphatidylserine, phosphatidic acid and salts thereof, glycercyl esters, sodium carboxymethylcellulose, bile acids

and salts thereof, cholic acid, deoxycholic acid, glycocholic acid, taurocholic acid, glycodeoxycholic acid, alkyl sulfonate, aryl sulfonate, alkyl phosphate, alkyl phosphonate, stearic acid and salts thereof, calcium stearate, phosphate, carboxymethylcellulose sodium, dioctyl sulfosuccinate, dialkyl esters of sodium sulfosuccinate, phospholipids, and calcium carboxymethylcellulose. However, the anionic surfactant is not limited thereto.

The cationic surfactant of the present specification may be selected from the group consisting of quaternary ammonium compounds, benzalkonium chloride, cetyltrimethylammonium bromide, chitosan, lauryldimethylbenzylammonium chloride, acyl carnitine hydrochloride, alkyl pyridinium halide, cetyl pyridinium chloride, cationic lipids, polymethylmethacrylate trimethylammonium bromide, sulfonium compounds, polyvinylpyrrolidone-2-dimethylaminoethyl methacrylate dimethyl sulfate, hexadecyltrimethyl ammonium bromide, phosphonium compounds, benzyl-di(2-chloroethyl)ethylammonium bromide, coconut trimethyl ammonium chloride, coconut trimethyl ammonium bromide, coconut methyl dihydroxyethyl ammonium chloride, coconut methyl dihydroxyethyl ammonium bromide, decyl trimethyl ammonium chloride, decyl dimethyl hydroxyethyl ammonium chloride bromide,  $(C_{12}-C_{15})$ dimethyl hydroxyethyl ammonium chloride,  $(C_{12}-C_{15})$ dimethyl hydroxyethyl ammonium chloride bromide, coconut dimethyl hydroxyethyl ammonium chloride, coconut dimethyl hydroxyethyl ammonium bromide, myristyl trimethyl ammonium methyl sulfate, lauryl dimethyl benzyl ammonium chloride, lauryl dimethyl benzyl ammonium bromide, lauryl dimethyl (ethenoxy)<sub>4</sub> ammonium chloride, lauryl dimethyl (ethenoxy)<sub>4</sub> ammonium bromide, N-alkyl  $(C_{12-18})$ dimethylbenzyl ammonium chloride, N-alkyl  $(C_{14-18})$ dimethyl-benzyl ammonium chloride, N-tetradecylidimethylbenzyl ammonium chloride monohydrate, dimethyl didecyl ammonium chloride, N-alkyl  $(C_{12-14})$ dimethyl 1-naphthylmethyl ammonium chloride, trimethylammonium halide alkyl-trimethylammonium salts, dialkyl-dimethylammonium salts, lauryl trimethyl ammonium chloride, ethoxylated alkyamidoalkylidalkylammonium salts, ethoxylated trialkyl ammonium salts, dialkylbenzene dialkylammonium chloride, N-didecyldimethyl ammonium chloride, N-tetradecylidimethylbenzyl ammonium chloride monohydrate, N-alkyl  $(C_{12-14})$ dimethyl 1-naphthylmethyl ammonium chloride, dodecyldimethylbenzyl ammonium chloride, dialkyl benzenalkyl ammonium chloride, lauryl trimethyl ammonium chloride, alkylbenzyl methyl ammonium chloride, alkyl benzyl dimethyl ammonium bromide,  $C_{12}$  trimethyl ammonium bromide,  $C_{15}$  trimethyl ammonium bromide,  $C_{17}$  trimethyl ammonium bromides, dodecylbenzyl triethyl ammonium chloride, poly-diallyldimethylammonium chloride, dimethyl ammonium chloride, alkyldimethylammonium halogenide, tricetyl methyl ammonium chloride, decyltrimethylammonium bromide, dodecyltriethylammonium bromide, tetradecyltrimethylammonium bromide, methyl triocetylammonium chloride, POLYQUAT 10, tetrabutylammonium bromide, benzyl trimethylammonium bromide, choline esters, benzalkonium chloride, stearalkonium chloride, cetyl pyridinium bromide, cetyl pyridinium chloride, halide salts of quaternized polyoxyethylalkylamines, "MIRAPOL" (polyquaternium-2), "Alkaquat" (alkyl dimethyl benzylammonium chloride, manufactured by Rhodia), alkyl pyridinium salts, amines, amine salts, imide azolinium salts, protonated quaternary acrylamides, methylated quaternary polymers, cationic guar gum, benzalkonium chloride, dodecyl trimethyl ammonium bromide, tri-

## 11

ethanolamine, and poloxamines. However, the cationic surfactant is not limited thereto.

The non-ionic surfactant of the present specification may be selected from the group consisting of SPAN 60, polyoxyethylene fatty alcohol ethers, polyoxyethylene sorbitan fatty acid esters, polyoxyethylene fatty acid esters, polyoxyethylene alkyl ethers, polyoxyethylene castor oil derivatives, sorbitan esters, glyceryl esters, glycerol monostearate, polyethylene glycols, polypropylene glycols, polypropylene glycol esters, cetyl alcohol, cetostearyl alcohol, stearyl alcohol, aryl alkyl polyether alcohols, polyoxyethylene-polyoxypolyethylene copolymers, poloxamers, poloxamines, methylcellulose, hydroxycellulose, hydroxymethylcellulose, hydroxyethylcellulose, hydroxypropylcellulose, hydroxypropylmethylcellulose, hydroxypropylmethylcellulose phthalate, non-crystalline cellulose, polysaccharides, starch, starch derivatives, hydroxyethyl starch, polyvinyl alcohol, triethanolamine stearate, amine oxide, dextran, glycerol, gum acacia, cholesterol, tragacanth, and polyvinylpyrrolidone.

The zwitterionic surfactant of the present specification may be selected from the group consisting of N-dodecyl-N, N-dimethyl-3-ammonio-1-propanesulfonate, betaine, alkyl betaine, alkylamido betaine, amido propyl betaine, cocoampho carboxy glycinate, sarcosinate aminopropionate, aminoglycinate, imidazolinium betaine, amphoteric imidazoline, N-alkyl-N,N-dimethylammonio-1-propanesulfonates, 3-cholamido-1-propyldimethylammonio-1-propanesulfonate, dodecylphosphocholine, and sulfo-betaine. However, the zwitterionic surfactant is not limited thereto.

FIG. 5 illustrates various examples of the cases where the second surfactant is positioned in two or more regions of the micelle, according to an exemplary embodiment of the present specification.

According to an exemplary embodiment of the present specification, the concentration of the first surfactant may be 1 time to 5 times the critical micelle concentration to the solvent. Specifically, the concentration of the first surfactant may be 2 times the critical micelle concentration to the solvent.

The critical micelle concentration (CMC) in the present specification means the lower limit of the concentration at which the surfactant forms a group (micelle) of molecules or ions in a solution.

The most important characteristics of the surfactant are that the surfactant tends to be adsorbed on an interface, for example, an air-liquid interface, an air-solid interface, and a liquid-solid interface. When the surfactants are free in the sense of not being present in an aggregated form, they are referred to as monomers or unimers, and when the unimer concentration is increased, they are aggregated to form small entities of aggregates, that is, micelles. The concentration may be referred to as the critical micelle concentration.

When the concentration of the first surfactant is less than 1 time the critical micelle concentration, the concentration of the first surfactant to be adsorbed on the first metal salt may be relatively decreased. Accordingly, the amount of core particles to be formed may also be entirely decreased. Meanwhile, when the concentration of the first surfactant exceeds 5 times the critical micelle concentration, the concentration of the first surfactant is relatively increased, so that metal nanoparticles which form a hollow core, and metal particles which do not form a hollow core may be mixed, and thus, aggregated. Accordingly, when the concentration of the first surfactant is 1 time to 5 times the critical micelle concentration to the solvent, the metal nanoparticles may be smoothly formed.

## 12

According to an exemplary embodiment of the present specification, the size of the metal nanoparticles may be adjusted by adjusting the first surfactant which forms the micelle, and/or the first and second metal salts which surround the micelle.

According to an exemplary embodiment of the present specification, the size of the metal nanoparticles may be adjusted by the chain length of the first surfactant which forms the micelle. Specifically, when the chain length of the first surfactant is short, the size of the micelle becomes small, and accordingly, the size of the metal nanoparticles may be decreased.

According to an exemplary embodiment of the present specification, the number of carbon atoms of the chain of the first surfactant may be 15 or less. Specifically, the number of carbon atoms of the chain may be 8 to 15. Alternatively, the number of carbon atoms of the chain may be 10 to 12.

According to an exemplary embodiment of the present specification, the size of the metal nanoparticles may be adjusted by adjusting the type of counter ion of the first surfactant which forms the micelle. Specifically, the larger the size of the counter ion of the first surfactant is, the weaker the binding force of the outer end portion of the first surfactant to the head portion is, so that the size of the micelle may be increased, and accordingly, the size of the metal nanoparticles may be increased.

According to an exemplary embodiment of the present specification, when the first surfactant is an anionic surfactant, the first surfactant may include  $\text{NH}_4^+$ ,  $\text{K}^+$ ,  $\text{Na}^+$ , or  $\text{Li}^+$  as the counter ion.

Specifically, the size of the metal nanoparticles may be decreased in the order of the case where the counter ion of the first surfactant is  $\text{NH}_4^+$ , the case where the counter ion of the first surfactant is  $\text{K}^+$ , the case where the counter ion of the first surfactant is  $\text{Na}^+$ , and the case where the counter ion of the first surfactant is  $\text{Li}^+$ .

According to an exemplary embodiment of the present specification, when the first surfactant is a cationic surfactant, the first surfactant may include  $\text{I}^-$ ,  $\text{Br}^-$ , or  $\text{Cl}^-$  as the counter ion.

Specifically, the size of the metal nanoparticles may be decreased in the order of the case where the counter ion of the first surfactant is  $\text{I}^-$ , the case where the counter ion of the first surfactant is  $\text{Br}^-$ , and the case where the counter ion of the first surfactant is  $\text{Cl}^-$ .

According to an exemplary embodiment of the present specification, the size of the metal nanoparticles may be adjusted by adjusting the size of the head portion of the outer end portion of the first surfactant which forms the micelle. Furthermore, when the size of the head portion of the first surfactant formed on the outer surface of the micelle is increased, the repulsive force between head portions of the first surfactant is increased, so that the micelle may be increased, and accordingly, the size of the metal nanoparticles may be increased.

According to an exemplary embodiment of the present specification, the aforementioned factors compositely act, so that the size of the metal nanoparticles may be determined.

According to an exemplary embodiment of the present specification, the metal salt is not particularly limited as long as the metal salt may be ionized in a solution to provide metal ions. The metal salt may be ionized in the solution state to provide a cation including a metal ion or an anion of an atomic group ion including the metal ion. The first metal salt and the second metal salt may be different from each other. Specifically, the first metal salt may provide a cation including a metal ion, and the second metal salt may provide

an anion of an atomic group ion including the metal ion. Specifically, the first metal salt may provide a cation of  $\text{Ni}^{2+}$ , and the second metal salt may provide an anion of  $\text{PtCl}_4^{2-}$ .

According to an exemplary embodiment of the present specification, the first metal salt and the second metal salt are not particularly limited as long as the first and second metal salts may be ionized in a solution to provide a metal ion or an atomic group ion including the metal ion.

According to an exemplary embodiment of the present specification, the first metal salt and the second metal salt may be each independently a salt of a metal selected from the group consisting of metals, metalloids, lanthanide metals, and actinide metals, which belong to Groups 3 to 15 of the periodic table.

Specifically, the first metal salt and the second metal salt are different from each other, and may be each independently a salt of a metal selected from the group consisting of platinum (Pt), ruthenium (Ru), rhodium (Rh), molybdenum (Mo), osmium (Os), iridium (Ir), rhenium (Re), palladium (Pd), vanadium (V), tungsten (W), cobalt (Co), iron (Fe), selenium (Se), nickel (Ni), bismuth (Bi), tin (Sn), chromium (Cr), titanium (Ti), gold (Au), cerium (Ce), silver (Ag), and copper (Cu).

More specifically, according to an exemplary embodiment of the present specification, the first metal salt may be a salt of a metal selected from the group consisting of ruthenium (Ru), rhodium (Rh), molybdenum (Mo), osmium (Os), iridium (Ir), rhenium (Re), palladium (Pd), vanadium (V), tungsten (W), cobalt (Co), iron (Fe), selenium (Se), nickel (Ni), bismuth (Bi), tin (Sn), chromium (Cr), titanium (Ti), cerium (Ce), silver (Ag), and copper (Cu), and more specifically, a salt of nickel (Ni).

More specifically, according to an exemplary embodiment of the present specification, the second metal salt may be a salt of a metal selected from the group consisting of platinum (Pt), ruthenium (Ru), rhodium (Rh), molybdenum (Mo), osmium (Os), iridium (Ir), rhenium (Re), palladium (Pd), vanadium (V), tungsten (W), cobalt (Co), iron (Fe), selenium (Se), nickel (Ni), bismuth (Bi), tin (Sn), chromium (Cr), titanium (Ti), gold (Au), cerium (Ce), silver (Ag), and copper (Cu). More specifically, the second metal salt may be a salt of a metal selected from a group consisting of platinum (Pt), palladium (Pd), and gold (Au), and more specifically, a salt of platinum (Pt).

According to an exemplary embodiment of the present specification, the first metal salt and the second metal salt may be each independently a nitrate, a halide such as chloride, bromide, and iodide, a hydroxide or a sulfate of the metal. However, the first metal salt and the second metal salt are not limited thereto.

According to an exemplary embodiment of the present specification, the molar ratio of the first metal salt to the second metal salt in the forming of the solution may be 1:5 to 10:1. Specifically, the molar ratio of the first metal salt to the second metal salt may be 2:1 to 5:1.

When the number of moles of the first metal salt is smaller than the number of moles of the second metal salt, it is difficult for a first metal ion to form a first shell including a hollow. Further, when the number of moles of the first metal salt is more than 10 times the number of moles of the second metal salt, it is difficult for a second metal ion to form a second shell surrounding a first shell. Therefore, the first and second metal ions may smoothly form a shell portion of the metal nanoparticles in the range.

According to an exemplary embodiment of the present specification, the shell portion may include: a first shell including the first metal ion; and a second shell including the second metal ion.

According to an exemplary embodiment of the present specification, the atomic percentage ratio of the first metal to the second metal in the shell portion may be 1:5 to 10:1. The atomic percentage ratio may be an atomic percentage ratio of the first metal of the first shell to the second metal of the second shell when the shell portion is formed of the first shell and the second shell. Alternatively, the atomic percentage ratio may be an atomic percentage ratio of the first metal to the second metal when the shell portion is formed of one shell including the first metal and the second metal.

According to an exemplary embodiment of the present specification, when the shell portion is formed of one shell including the first metal and the second metal, the first metal and the second metal may also be uniformly or non-uniformly mixed.

When the metal nanoparticle includes a hollow, the shell portion of the present specification may mean a region, which forms the metal nanoparticle, except for the cavity.

Alternatively, when the metal nanoparticle does not include a hollow, the shell portion may mean a region which forms the metal nanoparticle.

Alternatively, when the metal nanoparticle is a metal nanoparticle including one or more bowl-type particles, the shell portion may mean a region which forms the metal nanoparticle.

According to an exemplary embodiment of the present specification, the shell portion may be present in a state where the first metal and the second metal are gradated, the first metal may be present in an amount of 50% by volume or more or 70% by volume or more at a portion adjacent to the core in the shell portion, and the second metal may be present in an amount of 50% by volume or more or 70% by volume or more at a surface portion adjacent to the outer portion of nanoparticle in the shell portion.

According to an exemplary embodiment of the present specification, the forming of the solution may further include further adding a stabilizer.

The stabilizer may be, for example, a mixture of one or two or more selected from the group consisting of disodium phosphate, dipotassium phosphate, disodium citrate, and trisodium citrate.

According to an exemplary embodiment of the present specification, the forming of the metal nanoparticle may include further adding a non-ionic surfactant together with the reducing agent.

The non-ionic surfactant is adsorbed on the surface of the shell and thus serves to uniformly disperse the metal nanoparticles formed in the solution. Therefore, the non-ionic surfactant may prevent metal particles from being conglomerated or aggregated to be precipitated and allow metal nanoparticles to be formed in a uniform size. Specific examples of the non-ionic surfactant are the same as the above-described examples of the non-ionic surfactant.

According to an exemplary embodiment of the present specification, the solvent may be a solvent including water. Specifically, according to an exemplary embodiment of the present application, the solvent serves to dissolve the first metal salt and the second metal salt, and may be water or a mixture of water and a  $C_1$  to  $C_6$  alcohol, and more specifically, water. Since the preparation method according to the present specification does not use an organic solvent as the solvent, a post-treatment process of treating an organic

15

solvent in the preparation process is not needed, and accordingly, there are effects of reducing costs and preventing environmental pollution.

According to an exemplary embodiment of the present specification, the preparation method may be carried out at room temperature. The preparation method may be carried out at specifically 4° C. to 35° C., and more specifically 12° C. to 28° C.

The forming of the solution in an exemplary embodiment of the present specification may be carried out at room temperature, specifically 4° C. to 35° C., and more specifically 12° C. to 28° C. When an organic solvent is used as the solvent, there is a problem in that the preparation needs to be performed at a high temperature exceeding 100° C. Since the preparation may be carried out at room temperature, the present application is advantageous in terms of process due to a simple preparation method, and has a significant effect of reducing costs.

According to an exemplary embodiment of the present specification, the forming of the solution may be performed for 5 minutes to 120 minutes, more specifically for 10 minutes to 90 minutes, and even more specifically for 20 minutes to 60 minutes.

According to an exemplary embodiment of the present specification, the forming of the metal nanoparticle including the cavity by adding a reducing agent and/or a non-ionic surfactant to the solution may also be carried out at room temperature, specifically 4° C. to 35° C., and more specifically 12° C. to 28° C. Since the preparation method of the present specification may be carried out at room temperature, the method is advantageous in terms of process due to a simple preparation method, and has a significant effect of reducing costs.

The forming of the metal nanoparticle including the cavity may be performed by reacting the solution with the reducing agent and/or the non-ionic surfactant for a predetermined time, specifically for 5 minutes to 120 minutes, more specifically for 10 minutes to 90 minutes, and even more specifically for 20 minutes to 60 minutes.

According to an exemplary embodiment of the present specification, the reducing agent may have a standard reduction potential of -0.23 V or less.

The reducing agent is not particularly limited as long as the reducing agent is a strong reducing agent having a standard reduction potential of -0.23 V or less, specifically from -4 V to -0.23 V, and has a reducing power which may reduce the dissolved metal ions to be precipitated as metal particles. Specifically, the reducing agent may be at least one selected from the group consisting of NaBH<sub>4</sub>, NH<sub>2</sub>NH<sub>2</sub>, LiAlH<sub>4</sub>, and LiBEt<sub>3</sub>H.

When a weak reducing agent is used, a reaction speed is slow and a subsequent heating of the solution is required, so that it is difficult to achieve a continuous process, and thus, there may be a problem in terms of mass production, and particularly, when ethylene glycol, which is one of weak reducing agents, is used, there is a problem in that the productivity is low in a continuous process due to a decrease in flow rate caused by high viscosity. Therefore, when the reducing agent of the present specification is used, it is possible to overcome the problem.

According to an exemplary embodiment of the present specification, the preparation method may further include, after the forming of the metal nanoparticles including the cavity, removing a surfactant inside the hollow. The removing method is not particularly limited, and for example, a

16

method of washing the metal nanoparticles with water may be used. The surfactant may be an anionic surfactant and/or a cationic surfactant.

According to an exemplary embodiment of the present specification, the preparation method may further include, after the forming of the metal nanoparticle or after the removing of the surfactant inside the cavity, removing a cationic metal by adding an acid to the metal nanoparticle. When the acid is added to the metal nanoparticle in this step, a 3d band metal is eluted. The cationic metal may be specifically selected from the group consisting of ruthenium (Ru), rhodium (Rh), molybdenum (Mo), osmium (Os), iridium (Ir), rhenium (Re), palladium (Pd), vanadium (V), tungsten (W), cobalt (Co), iron (Fe), selenium (Se), nickel (Ni), bismuth (Bi), tin (Sn), chromium (Cr), titanium (Ti), cerium (Ce), silver (Ag), and copper (Cu).

According to an exemplary embodiment of the present specification, the acid is not particularly limited, and for example, it is possible to use an acid selected from the group consisting of sulfuric acid, nitric acid, hydrochloric acid, perchloric acid, hydroiodic acid, and hydrobromic acid.

According to an exemplary embodiment of the present specification, after the metal nanoparticles are formed, the solution including the metal nanoparticles may be centrifuged in order to precipitate the metal nanoparticles included in the solution. It is possible to collect only the metal nanoparticles separated after the centrifugation. If necessary, a process of sintering the metal nanoparticles may be additionally performed.

According to an exemplary embodiment of the present specification, it is possible to prepare metal nanoparticles having a uniform size of several nanometers. By methods in the related art, it was difficult to manufacture several nanometer-sized metal nanoparticles, and it was more difficult to prepare uniform-sized metal nanoparticles.

In an exemplary embodiment of the present specification, the metal nanoparticle may have an average particle diameter of 30 nm or less, more specifically 20 nm or less, or 12 nm or less, or 10 nm or less. Alternatively, the metal nanoparticle may have an average particle diameter of 6 nm or less. The metal nanoparticle may have an average particle diameter of 1 nm or more. When the metal nanoparticle has a particle diameter of 30 nm or less, there is a big advantage in that the nanoparticle may be used in various fields. Further, it is more preferred that the metal nanoparticle have a particle diameter of 20 nm or less. In addition, when the metal nanoparticle has a particle diameter of 10 nm or less or 6 nm or less, the surface area of the particle is further widened, so that there is an advantage in that the applicability of using the metal nanoparticles in various fields is further increased. For example, when the metal nanoparticles formed in the range of the particle diameter are used as a catalyst, the efficiency may be significantly increased.

According to an exemplary embodiment of the present specification, the average particle diameter of the metal nanoparticles means a value obtained by using a graphic software (MAC-View) to measure the diameters of 200 or more hollow metal nanoparticles, and measuring an average particle diameter through a statistical distribution obtained.

According to an exemplary embodiment of the present specification, the hollow metal nanoparticle may have an average particle diameter of 1 nm to 30 nm.

According to an exemplary embodiment of the present specification, the hollow metal nanoparticle may have an average particle diameter of 1 nm to 20 nm.

According to an exemplary embodiment of the present specification, the hollow metal nanoparticle may have an average particle diameter of 1 nm to 12 nm.

According to an exemplary embodiment of the present specification, the hollow metal nanoparticle may have an average particle diameter of 1 nm to 10 nm.

According to an exemplary embodiment of the present specification, the hollow metal nanoparticle may have an average particle diameter of 1 nm to 6 nm.

The shell portion in the metal nanoparticle in an exemplary embodiment of the present specification may have a thickness of more than 0 nm and 5 nm or less, more specifically more than 0 nm and 3 nm or less.

For example, when the metal nanoparticle includes a hollow, the average particle diameter is 30 nm or less, the shell portion may have a thickness of more than 0 nm and 5 nm or less, and more specifically, the metal nanoparticle has an average particle diameter of 20 nm or less or 10 nm or less, and the shell portion may have a thickness of more than 0 nm and 3 nm or less. According to an exemplary embodiment of the present specification, the hollow of the metal nanoparticle may have a particle diameter of 1 nm to 10 nm, specifically 1 nm to 4 nm. Further, each shell may have a thickness of 0.25 nm to 5 nm, specifically 0.25 nm to 3 nm. The shell portion may also be a shell formed by mixing the first metal and the second metal, and may be a plurality of shells including a first shell and a second shell, which are separately formed by varying the mixture ratio of each of the first metal and the second metal. Alternatively, the shell portion may also be a plurality of shells including a first shell including only the first metal and a second shell including only the second metal.

According to an exemplary embodiment of the present specification, when the metal nanoparticle prepared by the preparation method includes a hollow, the volume of the hollow may be 50% by volume or more, specifically 70% by volume or more, and more specifically 80% by volume or more of the total volume of the metal nanoparticle.

An exemplary embodiment of the present specification provides a metal nanoparticle prepared by the preparation method.

According to an exemplary embodiment of the present specification, the metal nanoparticle may have a spherical shape or a shape including one or more bowl-type particles.

According to an exemplary embodiment of the present specification, the metal nanoparticle may be a hollow metal nanoparticle including: a hollow core portion; a shell portion including a first metal and a second metal; and a cavity extending from the outer surface of the shell portion to the hollow core in one or two or more regions of the shell portion. Specifically, the hollow metal nanoparticle may include one cavity.

Further, according to an exemplary embodiment of the present specification, the hollow metal nanoparticle may be a metal nanoparticle including a first metal and a second metal, in which the metal nanoparticle includes one or more cavities which are continuous from the outer surface thereof. Specifically, the cavity may pass through the metal nanoparticle. Alternatively, the cavity may be continuous from an outer surface of the metal nanoparticle to one region inside of the metal nanoparticle.

In addition, according to an exemplary embodiment of the present specification, the metal nanoparticle may be a metal nanoparticle including one or more bowl-type particles including a first metal and a second metal.

The metal nanoparticles prepared by the preparation method of the present specification may be used while

replacing existing nanoparticles in the field in which nanoparticles may be generally used. The metal nanoparticles of the present specification have much smaller sizes and wider specific surface areas than the nanoparticles in the related art, and thus may exhibit better activity than the nanoparticles in the related art. Specifically, the metal nanoparticles of the present specification may be used in various fields such as a catalyst, drug delivery, and a gas sensor. The metal nanoparticles may also be used as a catalyst, or as an active material formulation in cosmetics, pesticides, animal nutrients, or food supplements, and may also be used as a pigment in electronic products, optical elements, or polymers.

#### MODE FOR INVENTION

The present specification will be described in detail with reference to the Examples for specifically describing the present specification. However, the Examples according to the present specification may be modified in various forms, and it is not interpreted that the scope of the present application is limited to the Examples described in detail below. The Examples of the present specification are provided for more completely explaining the present specification to the person with ordinary skill in the art.

The TEM images in the drawings of the present specification illustrate a dark field and/or a bright field of TEM. The dark field TEM image shows a bright image because diffraction significantly occurred in a shell portion having a large mass when the electron bunches of TEM touched the metal nanoparticles. Further, a region with hollows of the nanoparticles is shown as a slightly dark image because the electron bunches of TEM are less diffracted. In addition, a region with cavities of the shell portion is shown as a black image because the electron bunches of TEM are permeated as they are.

#### [Example 1]—Preparation of Hollow Metal Nanoparticle Including Cavity

40  $\text{Ni}(\text{NO}_3)_2$  as a first metal salt,  $\text{K}_2\text{PtCl}_4$  as a second metal salt, ammonium lauryl sulfate (ALS) as a first surfactant, N-dodecyl-N,N-dimethyl-3-ammonio-1-propane sulfonate (DDAPS) as a second surfactant, and trisodium citrate as a stabilizer were added to distilled water to form a solution, and the solution was stirred for 30 minutes. In this case, the molar ratio of  $\text{K}_2\text{PtCl}_4$  to  $\text{Ni}(\text{NO}_3)_2$  was 1:3, ALS was 2 times the critical micelle concentration (CMC) to water, and DDAPS was  $\frac{1}{30}$  mole of ALS.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of  $14^\circ\text{C}$ .

60 A transmission electron microscope (TEM) image of the metal nanoparticles, which were prepared according to Example 1, is illustrated in FIG. 8.

#### [Example 2]—Preparation of Hollow Metal Nanoparticle Including Cavity

65  $\text{Ni}(\text{NO}_3)_2$  as a first metal salt,  $\text{K}_2\text{PtCl}_4$  as a second metal salt, ammonium lauryl sulfate (ALS) as a first surfactant,

19

sodium 1-heptanesulfonate (SHS) as a second surfactant, and trisodium citrate as a stabilizer were added to distilled water to form a solution, and the solution was stirred for 30 minutes. In this case, the molar ratio of  $K_2PtCl_4$  to  $Ni(NO_3)_2$  was 1:3, ALS was 2 times the critical micelle concentration (CMC) to water, and SHS was  $\frac{1}{10}$  mole of ALS.

Subsequently,  $NaBH_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

A transmission electron microscope (TEM) image of the metal nanoparticles, which were prepared according to Example 2, is illustrated in FIG. 9.

[Example 3]—Preparation of Hollow Metal Nanoparticle Including Cavity

$Ni(NO_3)_2$  as a first metal salt,  $K_2PtCl_4$  as a second metal salt, ammonium lauryl sulfate (ALS) as a first surfactant, sodium hexanesulfonate as a second surfactant, and trisodium citrate as a stabilizer were added to distilled water to form a solution, and the solution was stirred for 30 minutes. In this case, the molar ratio of  $K_2PtCl_4$  to  $Ni(NO_3)_2$  was 1:3, ALS was 2 times the critical micelle concentration (CMC) to water, and sodium hexanesulfonate was  $\frac{1}{10}$  mole of ALS.

Subsequently,  $NaBH_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

A transmission electron microscope (TEM) image of the metal nanoparticles, which were prepared according to Example 3, is illustrated in FIG. 10.

[Example 4]—Preparation of Hollow Metal Nanoparticle Including Cavity

$Ni(NO_3)_2$  as a first metal salt,  $K_2PtCl_4$  as a second metal salt, sodium dodecyl sulfate (SDS) as a first surfactant, N-dodecyl-N,N-dimethyl-3-ammonio-1-propane sulfonate (DDAPS) as a second surfactant, and trisodium citrate as a stabilizer were added to distilled water to form a solution, and the solution was stirred for 30 minutes. In this case, the molar ratio of  $K_2PtCl_4$  to  $Ni(NO_3)_2$  was 1:3, ALS was 2 times the critical micelle concentration (CMC) to water, and DDAPS was  $\frac{1}{10}$  mole of ALS.

Subsequently,  $NaBH_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

20

A transmission electron microscope (TEM) image of the metal nanoparticles, which were prepared according to Example 4, is illustrated in FIG. 11.

5 [Example 5]—Preparation of Metal Nanoparticle Including Cavity

$Ni(NO_3)_2$  as a first metal salt,  $K_2PtCl_4$  as a second metal salt, ammonium lauryl sulfate (ALS) as a first surfactant, SPAN 60 as a second surfactant, and trisodium citrate as a stabilizer were added to distilled water to form a solution, and the solution was stirred for 30 minutes. In this case, the molar ratio of  $K_2PtCl_4$  to  $Ni(NO_3)_2$  was 1:3, ALS was 2 times the critical micelle concentration (CMC) to water, and SPAN 60 was  $\frac{1}{10}$  mole of ALS.

Subsequently,  $NaBH_4$  as a reducing agent and polyvinyl pyrrolidone (PVP) as a non-ionic surfactant were added to the solution and the mixture was left to react for 30 minutes.

10 Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

15 A transmission electron microscope (TEM) image of the metal nanoparticles, which were prepared according to Example 5, is illustrated in FIG. 12.

20 [Example 6]—Preparation of Metal Nanoparticle Including Cavity

$Ni(NO_3)_2$  as a first metal salt,  $K_2PtCl_4$  as a second metal salt, ammonium lauryl sulfate (ALS) as a first surfactant, sodium 1-heptanesulfonate (SHS) as a second surfactant, and trisodium citrate as a stabilizer were added to distilled water to form a solution, and the solution was stirred for 30 minutes. In this case, the molar ratio of  $K_2PtCl_4$  to  $Ni(NO_3)_2$  was 1:3, and ALS was 2 times the critical micelle concentration (CMC) to water, and SHS was  $\frac{1}{5}$  mole of SDS.

25 Subsequently,  $NaBH_4$  as a reducing agent and polyvinyl pyrrolidone (PVP) as a non-ionic surfactant were added to the solution and the mixture was left to react for 30 minutes.

30 Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

35 A transmission electron microscope (TEM) image of the metal nanoparticles, which were prepared according to Example 6, is illustrated in FIG. 13.

45 [Example 7]—Preparation of Metal Nanoparticle Including Cavity

$Ni(NO_3)_2$  as a first metal salt,  $K_2PtCl_4$  as a second metal salt, sodium dodecyl sulfate (SDS) as a first surfactant, N-dodecyl-N,N-dimethyl-3-ammonio-1-propane sulfonate (DDAPS) as a second surfactant, and trisodium citrate as a stabilizer were added to distilled water to form a solution, and the solution was stirred for 30 minutes. In this case, the molar ratio of  $K_2PtCl_4$  to  $Ni(NO_3)_2$  was 1:3, SDS was 2 times the critical micelle concentration (CMC) to water, and DDAPS was  $\frac{1}{10}$  mole of SDS.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

A transmission electron microscope (TEM) image of the metal nanoparticles, which were prepared according to Example 7, is illustrated in FIGS. 14 and 15.

[Example 8]—Preparation of Metal Nanoparticle Including One or More Bowl-Type Particles

$\text{Ni}(\text{NO}_3)_2$  as a first metal salt,  $\text{K}_2\text{PtCl}_4$  as a second metal salt, sodium dodecyl sulfate (SDS) as a first surfactant, SPAN 60 as a second surfactant, and trisodium citrate as a stabilizer were added to distilled water to form a solution, and the solution was stirred for 30 minutes. In this case, the molar ratio of  $\text{K}_2\text{PtCl}_4$  to  $\text{Ni}(\text{NO}_3)_2$  was 1:3, SDS was 2 times the critical micelle concentration (CMC) to water, and SPAN 60 was  $\frac{1}{10}$  mole of SDS.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

A transmission electron microscope (TEM) image of the metal nanoparticles, which were prepared according to Example 8, is illustrated in FIG. 16.

[Example 9]—Preparation of Metal Nanoparticle Including One or More Bowl-Type Particles

$\text{Ni}(\text{NO}_3)_2$  as a first metal salt,  $\text{K}_2\text{PtCl}_4$  as a second metal salt, sodium dodecyl sulfate (SDS) as a first surfactant, SPAN 60 as a second surfactant, and trisodium citrate as a stabilizer were added to distilled water to form a solution, and the solution was stirred for 30 minutes. In this case, the molar ratio of  $\text{K}_2\text{PtCl}_4$  to  $\text{Ni}(\text{NO}_3)_2$  was 1:3, SDS was 2 times the critical micelle concentration (CMC) to water, and SPAN 60 was  $\frac{1}{30}$  mole of SDS.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the present application. The process of preparing the metal nanoparticles was carried out under the atmosphere of 14° C.

A transmission electron microscope (TEM) image of the metal nanoparticles, which were prepared according to Example 9, is illustrated in FIG. 17.

[Example 10]—Preparation of Metal Nanoparticle Including One or More Bowl-Type Particles

$\text{Ni}(\text{NO}_3)_2$  as a first metal salt,  $\text{K}_2\text{PtCl}_4$  as a second metal salt, sodium dodecyl sulfate (SDS) as a first surfactant,

triethanol ammonium dodecyl benzene sulfate as a second surfactant, and trisodium citrate as a stabilizer were added to distilled water to form a solution, and the solution was stirred for 30 minutes. In this case, the molar ratio of  $\text{K}_2\text{PtCl}_4$  to  $\text{Ni}(\text{NO}_3)_2$  was 1:3, SDS was 2 times the critical micelle concentration (CMC) to water, and triethanol ammonium dodecyl benzene sulfate was  $\frac{1}{30}$  mole of SDS.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

A transmission electron microscope (TEM) image of the metal nanoparticles, which were prepared according to Example 10, is illustrated in FIG. 18.

[Example 11]—Preparation of Metal Nanoparticle Including One or More Bowl-Type Particles

$\text{Ni}(\text{NO}_3)_2$  as a first metal salt,  $\text{K}_2\text{PtCl}_4$  as a second metal salt, sodium hexanesulfonate as a first surfactant, ammonium lauryl sulfate (ALS) as a second surfactant, and trisodium citrate as a stabilizer were added to distilled water to form a solution, and the solution was stirred for 30 minutes. In this case, the molar ratio of  $\text{K}_2\text{PtCl}_4$  to  $\text{Ni}(\text{NO}_3)_2$  was 1:3, and the molar concentration of ALS was  $\frac{2}{3}$  time the molar concentration of sodium hexanesulfonate.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the present application. The process of preparing the metal nanoparticles was carried out under the atmosphere of 14° C.

A transmission electron microscope (TEM) image of the metal nanoparticles, which were prepared according to Example 11, is illustrated in FIGS. 19 and 20.

[Example 12]—Preparation of Metal Nanoparticle Including One or More Bowl-Type Particles

$\text{Ni}(\text{NO}_3)_2$  as a first metal salt,  $\text{K}_2\text{PtCl}_4$  as a second metal salt, ammonium lauryl sulfate (ALS) as a first surfactant, sodium hexanesulfonate as a second surfactant, and trisodium citrate as a stabilizer were added to distilled water to form a solution, and the solution was stirred for 30 minutes. In this case, the molar ratio of  $\text{K}_2\text{PtCl}_4$  to  $\text{Ni}(\text{NO}_3)_2$  was 1:3, ALS was 2 times the critical micelle concentration (CMC) to water, and the molar concentration of sodium hexanesulfonate was the same as that of ALS as 1:1.

Subsequently,  $\text{NaBH}_4$  as a reducing agent and polyvinyl pyrrolidone (PVP) as a non-ionic surfactant were added to the solution and the mixture was left to react for 30 minutes.

Thereafter, the mixture was centrifuged at 10,000 rpm for 10 minutes to discard the supernatant in the upper layer, and then the remaining precipitate was re-dispersed in distilled water, and then the centrifugation process was repeated to prepare the metal nanoparticles of the specification of the

present application. The process of preparing the metal nanoparticles was carried out under the atmosphere of 14° C.

A transmission electron microscope (TEM) image of the metal nanoparticles, which were prepared according to Example 12, is illustrated in FIGS. 21 and 22.

The invention claimed is:

1. A method for fabricating metal nanoparticles, the method comprising:

forming a solution comprising: a solvent; a first metal salt which provides a first metal ion or an atomic group ion comprising the first metal ion in the solvent; a second metal salt which provides a second metal ion or an atomic group ion comprising the second metal ion in the solvent; a first surfactant which forms micelles in the solvent; and a second surfactant which forms micelles together with the first surfactant in the solvent; and

forming metal nanoparticles comprising a hollow core by adding a reducing agent to the solution,

wherein the first metal ion or the atomic group ion comprising the first metal ion and the second metal ion or the atomic group ion comprising the second metal ion form a shell portion of the metal nanoparticle.

2. The method of claim 1, wherein the first metal ion or the atomic group ion comprising the first metal ion has a charge opposite to a charge at an outer end portion of the first surfactant, and

the second metal ion or the atomic group ion comprising the second metal ion has a charge which is the same as the charge at the outer end portion of the first surfactant.

3. The method of claim 1, wherein the shell portion of the metal nanoparticle is formed in a micelle region which the first surfactant forms, and a cavity of the metal nanoparticle is formed in a micelle region which the second surfactant forms.

4. The method of claim 1, wherein a cavity is formed in one or two or more regions of the shell portion by adjusting a concentration, a chain length, a size of an outer end portion, or a type of charge of the second surfactant.

5. The method of claim 4, wherein the adjusting of the chain length of the second surfactant is adjusting the chain length of the second surfactant to be different from a chain length of the first surfactant.

6. The method of claim 4, wherein the adjusting of the type of charge of the second surfactant is adjusting the charge of the second surfactant to be different from a charge of the first surfactant.

7. The method of claim 1, wherein a concentration of the first surfactant is 1 time to 5 times a critical micelle concentration to the solvent.

8. The method of claim 1, wherein a molar concentration of the second surfactant is 0.01 time to 1 time a molar concentration of the first surfactant.

9. The method of claim 1, wherein the chain length of the second surfactant is 0.5 time to 2 times a chain length of the first surfactant.

10. The method of claim 1, wherein both the first surfactant and the second surfactant are an anionic or cationic surfactant.

11. The method of claim 1, wherein one of the first surfactant and the second surfactant is an anionic surfactant, and the other is a cationic surfactant.

12. The method of claim 1, wherein the first surfactant is an anionic surfactant or cationic surfactant, and the second surfactant is a non-ionic or zwitterionic surfactant.

13. The method of claim 1, wherein the number of carbon atoms of the chain of the first surfactant is 15 or less.

14. The method of claim 1, wherein the first surfactant is an anionic surfactant, and comprises  $\text{NH}_4^+$ ,  $\text{K}^+$ ,  $\text{Na}^+$ , or  $\text{Li}^+$  as a counter ion.

15. The method of claim 1, wherein the first surfactant is a cationic surfactant, and comprises  $\text{I}^-$ ,  $\text{Br}^-$ , or  $\text{Cl}^-$  as a counter ion.

16. The method of claim 1, wherein the first metal salt and the second metal salt are each independently a nitrate, a halide, a hydroxide or a sulfate of the metal.

17. The method of claim 1, wherein the solvent comprises water.

18. The method of claim 1, wherein the preparation method is carried out at room temperature.

19. The method of claim 1, wherein a molar ratio of the first metal salt to the second metal salt is 5:1 to 10:1.

20. The method of claim 1, wherein the metal nanoparticle has a particle diameter of 1 nm to 30 nm.

21. The method of claim 1, wherein the first metal ion and the second metal ion are each independently an ion of a metal selected from the group consisting of platinum (Pt); ruthenium (Ru); rhodium (Rh); molybdenum (Mo); osmium (Os); iridium (Ir); rhenium (Re); palladium (Pd); vanadium (V); tungsten (W); cobalt (Co); iron (Fe); selenium (Se); nickel (Ni); bismuth (Bi); tin (Sn); chromium (Cr); titanium (Ti); gold (Au); cerium (Ce); silver (Ag); and copper (Cu).

22. The method of claim 1, wherein the shell portion comprises: a first shell comprising the first metal ion; and a second shell comprising the second metal ion.

23. The method of claim 1, wherein the metal nanoparticle has a spherical shape or a shape comprising one or more bowl-type particles.

\* \* \* \* \*